

Oct. 14, 1941.

E. A. MATTESON ET AL

2,259,260

METHOD OF CLEANING STRIP

Filed Oct. 30, 1939

2 Sheets-Sheet 1



BY

INVENTORS  
ELWIN A. MATTESON  
KIEL B. BOWMAN

*Rickey & Wootton*  
ATTORNEYS

Oct. 14, 1941.

E. A. MATTESON ET AL

2,259,260

METHOD OF CLEANING STRIP

Filed Oct. 30, 1939

2 Sheets-Sheet 2



## UNITED STATES PATENT OFFICE

2,259,260

## METHOD OF CLEANING STRIP

Elwin A. Matteson and Kiel B. Bowman, Youngstown, Ohio, assignors to The Aetna Standard Engineering Company, Youngstown, Ohio, a corporation of Ohio

Application October 30, 1939, Serial No. 261,966

5 Claims. (Cl. 15—269)

This invention relates to metal cleaning and more particularly to an improved method of and apparatus for removing oil or the like from strip steel or other elongated metal articles.

In the cold rolling of strip steel oil is applied to the surfaces of the metal for purposes of lubrication and to prevent oxidization of the surface of the metal. This oil may be either mineral or vegetable, palm oil being commonly used, and its removal after completion of the rolling operation presents a serious problem particularly in connection with strip which is to be used for porcelain enameling or lithograph work.

After rolling the strip is usually annealed by heating to a sufficiently high temperature in an annealing furnace. If there is any oil on the surface of the metal or in the pores of the metal this oil will carbonize during the annealing operation, leaving particles of carbonaceous material in or on the metal. Such particles prevent the proper adherence of lithographic or enamel coatings and thus the complete removal of all oil from the surfaces of the strip is of great importance.

It has previously been proposed to pass the strip through an alkali bath. This results in removing a portion of the oil but does not sufficiently clean the surface to entirely prevent the formation of carbon particles during annealing. It has also been proposed to scrub the surface of the sheet with an alkali solution but this likewise does not properly remove the oil.

It is among the objects of our invention to provide an improved method of cleaning strip by means of hot alkali solutions whereby oil will be substantially entirely removed and whereby the strip may be passed through the solution at high speed without reducing the cleaning efficiency. Other objects of our invention include the provision of an improved strip cleaning procedure which is simple and economical and which can be operated continuously for long periods of time without excessive attention; and the provision of an improved apparatus for carrying out the steps of our strip cleaning method.

The above and other objects of our invention will appear from the following description of certain preferred embodiments thereof, reference being had to the accompanying drawings, in which:

Figure 1 is a diagrammatic side elevational view, partly in section, of an apparatus for carrying out our improved cleaning procedure, the apparatus including electrical means for heating the strip.

Figure 2 is a diagrammatic side elevational view, partly in section, of a strip cleaning apparatus adapted to carry out the steps of our method but omitting the electrical strip heating equipment.

Figure 3 is a plan view of the apparatus shown in Figure 2.

Referring particularly to Figure 1, a coil of strip 1, which has come from the cold rolling mill and has a coating of oil, is illustrated at the left hand side of the view. This strip passes through the alkali scrubber indicated generally at S and which includes four staggered supporting rolls 2, 3, 4 and 5, and four rotary scrubbing brushes 6, 7, 8 and 9. Adjacent each of the scrubbing brushes is a hot alkali supply pipe 10. The scrubbing brushes and the pipes 10 extend across the entire width of the strip and the pipes are provided with perforations or nozzles adapted to direct a plurality of high velocity jets of hot alkali against the surface of the strip adjacent the scrubbing brushes. As shown by the arrows in Figure 1, the direction of rotation of the scrubbing brushes 6, 7, 8 and 9 is preferably opposed to the direction of movement of the strip through the apparatus. It will be understood that suitable feed rolls will be provided to move the strip through the apparatus at the desired rate of speed but such rolls are not shown as they form no part of the present invention.

In the preferred operation of our invention hot alkali solution (for example, soda ash and/or other alkali in water) at a temperature of about 160° F. is discharged upon the strip through the pipes 10. The scrubbing brushes 6, 7, 8 and 9, and the hot alkali remove the surface oil from the strip as it passes through the unit S. However, the scrubbing operation usually does not completely remove the oil which has been absorbed into the pores of the metal and in order to remove this oil we pass the strip over a guide pulley 11 into the tank 12 containing a hot alkali bath 13. Guide rolls 14 maintain the strip submerged beneath the surface of the alkali and a roller 15 guides the strip at the exit end of the tank 12.

A hood 16, having an outlet 17, may be provided to collect and carry away vapors and fumes which arise from the bath 13. In order to maintain the hot alkali bath 13 at the desired temperature, i. e. from about 190° F. to 230° F., heating pipes 18 may be provided in the bottom of the tank 12 and heated by steam or other suitable heating source.

As the cleaning and emulsifying action of the hot alkali on the oil varies approximately as the

square of the temperature of the alkali bath, we provide means in the tank 12 for electrically heating the reach of strip which is submerged in the bath 13 to a temperature somewhat above the boiling point of the bath, for example, approximately 250° F. This heating of the strip as it passes through the alkali bath 13 causes the solution immediately adjacent the surface of the strip to boil actively and the accompanying heat and agitation materially increase and facilitate the emulsification and removal of oil from the pores of the metal.

In order to apply the necessary current to the strip we preferably employ the arrangement shown in Figure 1, although it will be understood by those skilled in the art that various other hook-ups and contact means may be employed. In Figure 1 a central electrode roller 19 engages the strip opposite the central guide roll 14. Suitable means, not shown in detail, are provided for holding the roll 19 in engagement with the strip and electrical connections extend from the roll 19 through the wall of the tank 12, an insulator being indicated at 20, to one terminal of the secondary 21 of the transformer T. The opposite terminal of the secondary 21 is grounded at 22 and electrical connections lead from said opposite end of the secondary to the strip engaging electrode rolls 23 and 24. These rolls are preferably located opposite the end guide rolls 14 and are held against the strip by any suitable mechanism. Conductors 25 and 26 lead to the secondary 21 of the transformer T and the contact rollers 23 and 24 and their electrical connections are grounded at 27 and 28 respectively.

The transformer T is adapted to reduce the normal line voltage to a low value, for example 6 volts, and sufficient current is applied from the center terminal roller 19 to each of the end terminals 23 and 24 to heat the reaches of the strip indicated at 1<sup>a</sup> and 1<sup>b</sup> up to approximately 250° F., as explained above.

It will be observed that by means of the scrubber S and the jets of hot alkali solution therein the temperature of the strip may be elevated substantially, for example to about 150° F. This heated strip then enters the bath 13 and its temperature need be raised only a relatively small amount in order to get it up to the preferred value, i. e. the point at which the alkali will boil when in contact with the strip, and thus insure the most effective emulsifying and removal of the oil from the pores of the metal. The scrubber S performs two functions therefore, first to remove the larger portion of the surface film of oil from the strip, and second to preheat the strip so that it may readily be brought up to the desired temperature in the emulsifying bath 13.

The scrubber action alone will remove surface oil but does not effectively remove oil from the pores of the metal. The immersion of a strip in a bath of alkali, without previous scrubbing of the strip, is also ineffective to remove the oil thoroughly because such immersion does not remove the relatively thick surface oil with sufficient rapidity to permit of practical operation. Our improved procedure in which the strip is first scrubbed and preheated by high velocity hot alkali jets and then passed through an even hotter alkali solution where the alkali has free access to the oil in the pores of the metal with the result that the oil in the pores is emulsified and floats to the surface of the bath from which it may be skimmed or otherwise removed, re-

sults in complete removal of all oil from the metal and the cleaned strip can be annealed and used for enameling or lithographing without trouble.

5 After passing out of the bath 13 and over the roller 15 the strip is preferably rinsed by means of high pressure water sprays in the rinser R. The water spray nozzles are indicated at 29 and guide rolls 30 direct the strip through the rinser. Immediately following the rinser is a dryer D of any suitable type which evaporates any rinse water remaining on the strip and the oil-free strip will emerge from the dryer ready to be annealed or otherwise processed.

15 A modified form of our invention is illustrated in Figures 2 and 3, in which the coil of strip 31 passes through a scrubber S', substantially similar to the scrubber S and comprising supporting rolls 32, brushes 33 and high pressure hot alkali jets 34. The hot alkali tank 35 containing heating pipes 36 and the strip is guided by rollers 37, 38, 39 and 40 so that it passes below the surface of the alkali bath 41 for a distance sufficient to permit the hot alkali bath to emulsify the oil which remains in the pores of the metal after the scrubbing operation is carried out in the unit S'. In this form of our invention the electrical heating of the strip as it passes through the hot alkali bath 41 is not employed as, in some instances and with some types of oil, the additional emulsifying and cleaning action caused by the active boiling of the alkali solution immediately at the surface of the strip may not be required. The washer or rinser R' is substantially similar to the rinser R and the dryer D' is the equivalent of the dryer D.

20 The alkali baths 13 and 41 may be maintained substantially at the boiling temperature of the solution, i. e. approximately 220° F., by means of superheated steam in the pipes 36 and we have found that the cooperative results of this bath with the combined scrubbing and preheating which occurs in the scrubber S and which removes the surface film of oil in such a manner that the hot bath of alkali in the tank can have access to the oil in the pores of the metal, produces cleaning results impossible to obtain with previously proposed methods and apparatus. Our electrical heating procedure for raising the strip 25 to a temperature higher than the boiling point 30 of the solution permits an agitation and extremely effective release of emulsified oil from the pores of the strip in the bath.

25 The entire system is adapted for continuous operation and, although we have described in considerable detail the illustrated embodiments of our improved apparatus and certain preferred procedures for carrying out our method, it will be understood by those skilled in the art that variations and modifications may be made without departing from the spirit of our invention. We do not, therefore, wish to be limited to the particular form herein described but claim as our invention all embodiments thereof coming within the scope of the appended claims.

60 We claim:

1. In the cleaning of strip metal or the like, a process which includes the steps of moving the strip in the direction of its length, preheating the moving strip to between 100° F. and 200° F., scrubbing both sides of said strip with a hot alkali solution whereby surface oil is removed, passing said preheated moving strip into an alkali bath, maintaining the temperature of the bath between 190° F. and 230° F., permitting

said moving preheated strip to remain in the bath long enough to emulsify and remove oil from the pores of the metal surfaces, removing said strip from the bath, and subjecting said strip to a water rinse.

2. A process of continuously cleaning longitudinally moving strip metal or the like which includes the steps of preheating the moving strip and causing high velocity hot alkali solution to impinge upon both sides of the moving strip, scrubbing the surfaces of both sides of the strip in the presence of said hot alkali solution whereby surface oil is removed from the strip, passing said preheated strip into and through a hot alkali bath, maintaining the temperature of said bath between about 190° F. and 230° F. whereby oil in the pores of the surface of said strip is emulsified and removed, and rinsing said strip to remove the alkali therefrom.

3. A process of continuously cleaning longitudinally moving strip metal which includes the steps of passing the strip through an alkali bath, and, while the strip is submerged in the bath, generating heat in the strip itself whereby both

10 ing of the alkali bath will occur adjacent the surfaces of the strip.

4. A process of continuously cleaning longitudinally moving strip metal which includes the 5 steps of passing the strip through an alkali bath, and, while the strip is submerged in the bath, causing an electric current to flow in a reach of the strip which is submerged in said bath whereby said reach of strip is heated to a temperature above about 200° F.

5. A process of continuously cleaning longitudinally moving strip metal which includes the 15 steps of causing high velocity jets of alkali solution at a temperature of 150° F. or higher to impinge against both sides of the moving strip whereby said strip is preheated, scrubbing both sides of said strip in the presence of said hot alkali solution, passing said preheated strip through a hot alkali bath, maintaining the temperature of said bath between about 190° F. and 230° F., generating heat by electrical resistance in the reach of strip in said alkali bath, and rinsing said strip to remove alkali therefrom.

ELWIN A. MATTESON,  
KIEL B. BOWMAN.